

## UNITED STATES PATENT OFFICE

CORNELIS WARNARDUS ZAHN, OF HELMOND, NETHERLANDS, ASSIGNOR TO NAAMLOOZE  
VENNOOTSCHAP: J. A. CARP'S GARENFABRIEKEN, OF HELMOND, NETHERLANDS

## METHOD OF PREPARING DULL ARTIFICIAL SILK

No Drawing. Application filed July 31, 1929, Serial No. 382,599, and in the Netherlands May 24, 1929.

The invention relates to a method of preparing dull artificial silk, from cellulose esters, such as acetate silk, and especially from regenerated cellulose, such as viscose-  
5 and ammoniacal copper oxide silk.

For obtaining a dull lustre of artificial silk various methods are applied.

1. The spinning solution, e. g. the viscose solution, is prepared with some ingredient, 10 which causes the spun thread to look dull. In this case the dull lustre is inherent to the fibre. The chemicals used form a homogeneous mixture with the regenerated cellulose.

15 2. The normally prepared spinning solution is spun and the silk obtained is submitted to a subsequent treatment which causes a precipitate to settle on the fibre, 20 causing the silk to look dull. This precipitate may consist of an insoluble salt, e. g. an inorganic salt like barium sulphate or an organic salt, such as fatty acid salts of aluminium.

25 3. The fibre is submitted to a swelling process by means of concentrated sulphuric or phosphoric acid, chloride of zinc, and such like substances.

30 4. The fibre is impregnated with titanic salts, upon which the bath is heated; finally the titanic salt is converted into hydroxide by means of heating in an autoclave.

According to the invention it has been found that a lasting aftertreatment which, 35 like the method mentioned sub 4 is based on a hydrolysis, may be obtained by treating the silk with a solution of suitable silicofluorides in water which are capable of separating silicic acid when heated. A very suitable silicofluoride for this purpose is magnesiumsilicofluoride ( $MgSiF_6 \cdot 6H_2O$ ). This silicofluoride is easily soluble in cold water (1:1.5) and gradually separates silicic acid when heated, the silicic acid being dissolved again after cooling.

45 Now this process is based on the principle that the silicic acid separated by heating is partly incorporated into the silk, in such a way that it cannot be washed away, when the silk is rinsed with water, or treated with 50 diluted acids or soap solutions.

The silk to be treated is introduced into a cold solution of the silicofluoride; then the temperature of the bath is gradually raised. After a sufficiently long time the silk is taken from the bath, and thoroughly rinsed with 55 water. The resulting silk can immediately be dyed or dried.

The product obtained in this way is a dull, milky white silk, which may easily be moistened, and submitted to a further treatment. 60 The silk has decreased about 10% in strength but this may be remedied to a certain extent by adding a little ammonia to the silicofluoride solution. This results moreover in the solution being quite clear again, when cooled 65 down, and it may then be used for a following treatment. When rinsed with water, and treated with diluted acids the silk is very 70 resistant. It is sufficiently proof against soap solutions of 50-60° C.

The dull silk obtained according to the invention is, however, not quite proof against a hypochlorite solution, as by a treatment of the silk with such a solution the lustre is 75 partly restored.

The circumstance that the treatment may be effected in one single bath and that the silk need only be slightly manipulated, is a great advantage of the process described, and is very useful at the moment of sorting. 80

The process is illustrated by the following example:

100-400 g. of magnesium silicofluoride are dissolved in 10 L. of cold water. 500 g. of dry silk are introduced into this solution, and left for about 10 minutes in the same. Then the temperature of the bath is gradually raised to 70°-90° C. and the silk is allowed to remain about another 10 minutes in the bath. The silk need only be stirred round a few times. This stirring may be further reduced, when curved sticks are used, submerging the silk altogether in the bath. 90

After the treatment the silk is thoroughly rinsed and is then ready for further treatment, drying or dyeing. 95

I claim:

1. The process of providing artificial silk with a dull lustre which comprises introducing the finished silk into a solution containing 100

ing a silico fluoride and heating the said solution.

5 2. The process of providing artificial silk with a dull lustre which comprises introducing the finished silk into a solution containing magnesium silico fluoride and heating the said solution.

In testimony whereof I affix my signature.

**10****Dr. CORNELIS WARNARDUS ZAHN.****15****20****25****30****35****40****45****50****55****60**